

Dec. 11, 1951

C. A. SOUTHWICK, JR

2,578,324

DESIDCANT POUCH

Filed Sept. 7, 1945



Fig. 2



Fig. 3



Fig. 4



Fig. 5



INVENTOR.

Charles A. Southwick, Jr.,  
BY

Cromwell, Griggs & Warden  
attys

## UNITED STATES PATENT OFFICE

2,578,324

## DESICCANT POUCH

Charles A. Southwick, Jr., Mount Vernon, Ohio,  
assignor to Shellmar Products Corporation,  
Mount Vernon, Ohio, a corporation of Delaware

Application September 7, 1945, Serial No. 614,985

3 Claims. (Cl. 183—4.8)

1

The present invention relates to improvements in coated sheet material. More particularly, it pertains to a water vapor permeable sheet material having a heat-sealable coating thereon with a water vapor permeable material embedded in the coating, thereby providing a combined heat-sealable structure having increased water vapor transmission characteristics, and the provision of such an article is a principal object of the invention.

More specifically, it is an object of the invention to provide a fibrous base sheet which has a relatively high rate of water vapor permeability, a heat-sealable coating on one surface of the fibrous sheet, a finely divided fibrous material, which also has a relatively high rate of water vapor permeability, embedded in the coating in such a manner that its fibers extend throughout the coating so that some of them are exposed at the coating surface and some of them are exposed to contact with the fibrous base sheet, the fiber impregnated coating being rendered increasingly water vapor permeable by the embedded fibrous material whereby the water vapor transmission characteristic of the combined construction is considerably enhanced.

Yet more specifically, it is an object of the invention to provide a package made of sheets of fibrous container material having a relatively high rate of water vapor permeability, a heat-sealable coating on each of the sheets, and a finely divided fibrous material which also has a relatively high rate of water vapor permeability which is embedded within the coating, the sheets being arranged into container or pouch formation with the coating material on the inside and being heat-sealed where it is in face-to-face seam forming relationship, the fibrous embedded material in the coating strengthening the seam structure, and the container, or pouch, being provided with a desiccant, whereby water vapor readily can be absorbed through the walls thereof at an increased rate.

Other objects of the invention will in part be obvious and will in part appear hereinafter.

The invention accordingly comprises an article of manufacture possessing the features, properties, and the relation of elements which will be exemplified in the article hereinafter described and the scope of the application of which will be indicated in the claims.

For a fuller understanding of the nature and objects of the invention reference should be had to the following detailed description taken in connection with the accompanying drawings, in which:

2

Fig. 1 is a diagrammatic illustration of an apparatus for practicing a method embodying the invention of combining fibrous sheets by means of a coating composition so that one sheet is embedded within the coating;

Fig. 2 is a perspective view of a fragment, on an enlarged scale, of a fibrous coated sheet with another sheet embedded in the coating;

Fig. 3 is a plan view of a type of container, or pouch, made from such coated sheets with a corner portion removed to show the contents;

Fig. 4 is an end elevational view with a portion broken away, and partly in section, illustrating the pouch, or container, of Fig. 3; and

Fig. 5 is a fragmentary portion taken through the heat-sealed seam construction, for example, on the line 5—5 of Fig. 3, on an enlarged scale further illustrating another feature of the invention.

Pouches, or containers, made from coated container material embodying the present invention, when filled with a desiccant such as silica gel, are useful when placed in bags or containers of all sizes protectively covering mechanisms or instruments where it is desirable hermetically to package them and to keep them free from moisture. During the initial stage of wrapping or packaging such articles, and after they are hermetically sealed in the package, it is essential to remove as much moisture as possible. This previously has been done by putting cloth bags containing desiccants, such as silica gel, therein to absorb the moisture or vapor confined within the container. However, such containers have proved to be expensive because they are hand-made and require special linings to render them sift proof and dust tight and the walls have not had the necessary high moisture vapor transmissive characteristics to enable them rapidly to transmit moisture.

The foregoing difficulties and other disadvantages have been overcome by means of the present invention wherein a coated material, for making pouches containing a desiccant, is utilized in which water vapor transmission rate, sift proofness and durability characteristics can be provided in a more economical and facile manner.

Referring more particularly to Fig. 1 of the drawings there is illustrated a suitable apparatus for practicing the present invention. A mill roll 10, for example, of kraft paper is unwound to provide a web 11 which passes around an idler roller 12. Running between the idler roller 12 and the web 11 is another web 13 coming off a mill roll 14, for example, of tissue paper. An

example of the kraft paper employed would be a 30 pound weight per ream. An example of the tissue would be a 10 pound weight per ream.

Both webs 11 and 13, after they pass around the idler roller 12, form a double web 15 which passes around idler rollers 16, 17 and 18. The double web is then run around a drum, or cylinder, 19 rotating in a bath of heat-sealable adhesive coating 20 in a trough 21. A suitable coating material, for example, is a vinyl chloride acetate copolymer, or a butyral lacquer. The double web 15 is passed around the drum 19. The heavy kraft web 11 lies against the drum surface and the kraft tissue web 13 is exposed to the coating material. As the drum is rotated, the web 11 becomes coated and the tissue is embedded in, or impregnated with the coating of heat-sealable material.

As the combined web travels toward the top of the drum the excess coating material is caused to flow back into the tank because of the pressure of a squeeze roller 22. Any suitable leveling device 23 can be positioned above the coated web 11 carrying the tissue embedded fibrous material and this leveling device knocks down ridges and irregularities in the surface of the coating.

In Fig. 2 the kraft sheet 11 illustrates the numerous fibers which transmit to the sheet its water vapor permeable characteristics. It will be appreciated from the illustration that the coating material 20 has embedded therein the fibrous tissue web 13 and that the ends of the tissue material tend to become exposed at the upper surface of the coating as indicated in the drawings. At the same time these tissue fibers will lie adjacent to or in contact with the fibers of the kraft material 11. The fibers of the tissue 13 provide numerous means of communication for the transmission of water vapor to the kraft sheet 11.

It is significant that the coating material 20 is also broken up by the fibers of the tissue 13 additionally to provide numerous minute channels communicating with the kraft sheet 11 for transmission of water vapor. In this manner a coated sheet is provided which does not carry an adhesively fixed sheet of fibrous material but a thin fibrous sheet which provides a wick action for moisture vapor transmission. At the same time the heat-sealable material strengthens the kraft paper but because of the fact that it is broken up by the numerous tentacles of the tissue, it also is rendered very porous and the combined construction has enhanced water vapor transmission characteristics. Furthermore, the heat-sealing characteristics of the coating material is not impaired. Indeed, because of the fibrous tentacles of the tissue 13 embedded in the coating material, two coated surfaces of such a sheet, when brought together under heat and pressure, will combine interlocking to provide a sheet having added strengthening and sealing characteristics in the seam area.

It should be understood that the material with which the coating is loaded need not necessarily be a tissue such as that above described, but preferably such a material is utilized. Any suitable flocculent material, such as cotton linters, or the like, can be blown or otherwise impregnated into the coating material after it has been applied to the base sheet of fibrous material 11.

It is within the contemplation of the invention that other suitable materials for loading the coating material can also be utilized as, for ex-

ample, a sheet of very finely woven cloth fabric.

A package, or pouch, made from two sheets of material similar to those above described is illustrated in Figs. 3 and 4. A desiccant, such as silica gel, is placed in a portion of the pouch and the marginal edges thereof heat-sealed under heat and pressure, the coated surfaces, of course, being in face-to-face relationship.

An illustration of a heat-sealed seam construction embodying the invention is shown in Fig. 5 and it will be appreciated that the fibers in the coating material of such a seam will be intertwined and interlocking engaged with each other where they are buried or fused in the heat-sealable coating.

Another feature of importance is that after the coating operation and during the drying of the coated web impregnated with the tissue or like material, there is an increased rate of solvent migration and evaporation from the coating because of the wicking action of the embedded tissue fibers, many of which are exposed at the surface of the coating. In other words, such a web can be coated and run at high speed and production facilities can greatly be increased.

It will thus be seen that the objects hereinbefore set forth may readily and efficiently be attained, and since certain changes may be made in the above article and different embodiments of the invention could be made without departing from the scope thereof, it is intended that all matter contained in the above description or shown in the accompanying drawings shall be interpreted as illustrative and not in a limiting sense.

Having described my invention, what I claim as new and desire to secure by Letters Patent, is:

1. A package comprising sheets of fibrous container material having a relatively high rate of water vapor permeability, an overall coating on each of said fibrous sheets, which coating is a heat-sealable material, a finely divided fibrous material which also has a relatively high rate of water vapor permeability being embedded within and evenly distributed throughout said coating so that fibers of said last named fibrous material extend completely throughout said coating, some of which fibers are exposed at the coating surface and some of which are exposed to contact with fibers of said fibrous sheets of container material, said coating being rendered water vapor permeable by said embedded fibrous material, said sheets being arranged into container formation with the coating material on the inside and being heat-sealed where the sheets are in face-to-face seam forming relationship with said fibrous embedded material in said coating thereby strengthening said seam structure, and said container being provided with a desiccant to provide a package whereby water vapor readily can be absorbed through the walls thereof, said combined container structure having a high water vapor transmission rate.

2. A package as defined in claim 1, and wherein in said fibrous material consists of a sheet of tissue embedded in said coating material.

3. A package as defined in claim 1, and wherein in said fibrous material consists of overall dispersion of linter material embedded within said coating.

CHARLES A. SOUTHWICK, JR.

(References on following page)

## REFERENCES CITED

The following references are of record in the file of this patent:

## UNITED STATES PATENTS

| Number    | Name        | Date          | Number      |
|-----------|-------------|---------------|-------------|
| 25,192    | Goodyear    | Aug. 23, 1859 | 2,306,400   |
| 1,906,671 | Thunert     | May 2, 1933   | 2,317,730   |
| 2,039,312 | Goldman     | May 5, 1936   | 2,430,459   |
| 2,210,862 | Tronstad    | Aug. 6, 1940  | 5 2,441,477 |
| 2,277,050 | Reed et al. | Mar. 24, 1942 | 10 437,139  |

| Name           | Date          |
|----------------|---------------|
| Menzel         | Dec. 29, 1942 |
| Calvert        | Apr. 27, 1943 |
| Farrell et al. | Nov. 11, 1947 |
| Farrell        | May 11, 1948  |

## FOREIGN PATENTS

| Country       | Date          |
|---------------|---------------|
| Great Britain | May 14, 1925  |
| Great Britain | Oct. 25, 1935 |